

## [54] CORROSION INHIBITORS

[75] Inventors: Eugene V. Hort, Wayne; Lowell R. Anderson, Morristown; Dru W. Alwani, Wayne, all of N.J.

[73] Assignee: GAF Corporation, New York, N.Y.

[21] Appl. No.: 301,667

[22] Filed: Sep. 14, 1981

[51] Int. Cl.<sup>3</sup> ..... C23F 11/14; C23F 11/04

[52] U.S. Cl. ..... 252/392; 106/14.13; 106/14.15; 252/8.55 C; 252/8.55 E; 422/12; 422/16

[58] Field of Search ..... 252/392, 8.55 C, 8.55 E; 106/14.13, 14.15; 422/12, 16

## [56] References Cited

## U.S. PATENT DOCUMENTS

3,079,345 2/1963 Monroe et al. ..... 252/390  
3,107,221 10/1963 Harrison et al. ..... 252/390

3,231,507 1/1966 Beale et al. ..... 252/396  
3,382,179 5/1968 Keeney et al. ..... 252/390  
3,428,566 2/1969 Herman et al. ..... 252/388  
3,705,106 12/1972 Muzyckzo et al. ..... 252/392  
3,772,208 11/1973 Tedeschi et al. ..... 252/855 E  
3,779,935 12/1973 McDougall et al. ..... 252/392  
3,802,890 4/1974 Keeney ..... 252/390  
3,816,322 6/1974 Griffin et al. ..... 252/392

Primary Examiner—Irwin Gluck

Attorney, Agent, or Firm—Marilyn J. Maué; J. Gary Mohr; Joshua J. Ward

[57]

## ABSTRACT

An aqueous composition for inhibiting the corrosion of metals placed therein is described. The composition comprises a non-oxidizing acid and, as a corrosion inhibitor, an effective amount of a 3-dialkylamino-3-(substituted phenyl)-prop-1-yne.

26 Claims, No Drawings

## CORROSION INHIBITORS

## BACKGROUND OF THE INVENTION

## 1. Field of the Invention

This invention relates to compositions for inhibiting the corrosion of metals placed therein, and to novel acetylenic amines for such use.

## 2. Description of the Prior Art

In the field of oil-well acidizing, it is necessary to use inhibitors to prevent corrosion of the oil-well equipment by the acid solutions employed. Many different acetylenic amines have been proposed or used as corrosion inhibitors for oil-well acidization; see e.g. U.S. Pat. Nos. 2,997,507; 3,079,345; 3,107,221; 3,231,507; 3,268,524; 3,268,583; 3,382,179; 3,428,566; 3,496,232; 3,705,106; 3,772,208; 3,779,935; 3,802,890; 3,816,322; and 4,002,694; and the articles entitled "Ethynylation" by W. Reppe, et al. Ann. Chem. 59B, 1-224 (1955); and "Acetylenic Corrosion Inhibitors", by Foster et al., Ind. and Eng. Chem., 51, 825-8 (1959).

Nonetheless, there has been a continuing search for new materials which are highly effective in such application. More particularly, it is desired to provide new and improved corrosion inhibitors which are particularly advantageous in commercial use to prevent corrosion of metals in highly acid solutions, even after prolonged periods of use, which have a low vapor pressure and relatively high stability so that they can be employed at the high temperatures which prevail in modern deep drilling operations, which function effectively at low concentrations, and which are relatively inexpensive to make.

## SUMMARY OF THE INVENTION

What is described herein is an aqueous composition for inhibiting the corrosion of metals placed therein which comprises: (a) a 3-dialkylamino-3-(substituted phenyl)-prop-1-yne compound as a corrosion inhibitor having the formula:



where

R<sub>1</sub> and R<sub>2</sub> are independently alkyl C<sub>1</sub>-C<sub>8</sub>;

R<sub>3</sub> is independently halo, alkyl C<sub>1</sub>-C<sub>8</sub> or alkoxy C<sub>1</sub>-C<sub>8</sub>; and

n is 1 or 2; and

(b) a non-oxidizing acid.

In the preferred form of the invention, both R<sub>1</sub> and R<sub>2</sub> are alkyl C<sub>2</sub>-C<sub>6</sub>; R<sub>3</sub> is 2-halo; and n is 1. A preferred compound is 3-dibutylamino-3-(2-chlorophenyl)-prop-1-yne, having the formula:



The compounds of the invention are made by a catalytic ethynylation reaction, followed by purification, such as by molecular distillation of the crude reaction product under vacuum, or liquid chromatography.

## DETAILED DESCRIPTION OF THE INVENTION

The catalytic ethynylation reaction between a dialkylamine, a substituted benzaldehyde, and acetylene, to produce the 3-dialkylamino-3-(substituted phenyl)-prop-1-yne, proceeds as follows:



where R<sub>1</sub>, R<sub>2</sub>, R<sub>3</sub> and n are as defined above.

The reaction is carried out in the presence of an ethynylation catalyst, such as is used for commercial preparation of butynediol; see, e.g. U.S. Pat. Nos. 3,920,759; 4,117,248; and 4,119,790. The preferred catalyst is a complex cuprous acetylidyde prepared from a precursor containing about 5 to 35% by weight of copper, and 2-3% by weight of bismuth, as the oxides, on a magnesium silicate carrier. However, many other ethynylation catalysts and carriers known in the art may be used as well.

The ethynylation reaction can be run under low or high pressure conditions, i.e. a partial pressure of acetylene, as is used for butynediol, generally from about 0.1 atmosphere to 20 or more atmospheres, either in a stirred reactor with a slurried catalyst, or in a fixed bed, through which the acetylene and the solution are passed.

The ethynylation process preferably is run in a solvent in which the reactants are at least partially soluble. An organic solvent which is inert to the reaction may be used advantageously; preferably it is also volatile so that it can be easily separated from the reaction product by distillation. Alcohols, hydrocarbons and other organic solvents may be used for this purpose. A preferred organic solvent is either dry or aqueous isopropanol.

Water also is a suitable solvent; however, water does not completely dissolve the reactants, and it wets the catalyst, which interferes with wetting by the organic reactants. The ethynylation reaction rate thus is slower in water than in an organic solvent which forms a single liquid phase. Mixtures of an organic solvent and water may be used, most suitably those which give a single reacting liquid phase.

In a typical run, a charge is made of the reactants in a molar ratio of about 1:1 of the dialkylamine and substituted benzaldehyde. The charge then is heated to a temperature of about 70° to 115° C., preferably 85° to 105° C., and acetylene is introduced and maintained at the desired pressure. The reaction then is carried out for from less than 1 to 36 hours, generally for about 0.2 to 8 hours.

The crude reaction product then is separated from the catalyst, where necessary, stripped of solvent by rotary evaporation under reduced pressure and the crude reaction mixture is purified by fractional distillation under vacuum. Gas chromatographic (GC) assay indicates that the isolated compounds have a purity of at least 85%, and usually 95% or more. Some decomposition of the compound may occur, however, at the temperature of the assay.

The purified compound may be characterized by its IR and NMR spectra. The IR spectrum shows the presence of a strong sharp C—H stretching absorption band at about  $3320\text{ cm}^{-1}$ , attributable to the ethynyl group, and an absence of carbonyl absorption in the region of  $1600\text{--}1700\text{ cm}^{-1}$ . The NMR spectrum shows distinctive absorptions related to the



portion of the molecule. The C-1 proton is evident by a doublet at  $3.1\text{--}5.2\delta$  due to coupling of the C-3 proton with the C-1 proton. The C-3 proton also shows up as a doublet for the same reason; however, at  $2.0\text{--}3.0\delta$ . In addition, the NMR spectrum of the compounds herein reveals the absence of both an aldehyde proton absorption, which is present in the starting material at  $9\text{--}10\delta$ , and any N—H absorption.

The crude ethynylation reaction product is a complex mixture which contains predominately 3-dialkylamino-3-(substituted phenyl)-prop-1-yne; in addition, it may contain some 3-dialkylaminobutyne, e.g.  $\text{R}_1\text{R}_2\text{NCH}(\text{CH}_3)\text{C}\equiv\text{CH}$ , and, depending upon reaction conditions, unreacted starting materials, and lesser amounts of other materials.

The corrosion-inhibiting compositions of the invention may be used at varying concentrations. What is an effective amount in a particular application will depend upon local operating conditions. For example, the temperature and other characteristics of the acid corrosion system will have a bearing upon the amount of inhibitor to be used. The higher the temperature and/or the higher the acid concentration, the greater is the amount of corrosion inhibitor required to give optimum results. In general, however, it has been found that the corrosion inhibitor composition of the invention should be employed at a concentration of between 0.01 and 2%, preferably between 0.01% and 1.2%, by weight of the aqueous acidic solution, although higher concentrations can be used when conditions make them desirable. An inhibitor concentration between 0.05% and 0.75% by weight is of the most general use, particularly at elevated temperatures, e.g. in the neighborhood of  $200^\circ\text{ F}$ .

The acidic solution itself can be dilute or concentrated as desired, and can be of any of the specific concentrations customarily used in treating metals, e.g. ferrous metals, or for operations involving contact of acidic solutions with such metals in oil-well acidizing. Generally the acid content is about 5 to 80%, and, in most operations of the character indicated, acid concentrations of 10-15% by weight are employed. Non-oxidizing inorganic acids are the most common acids used.

The invention will now be described in more detail by the following examples which are for illustration only, and not by way of limitation.

#### EXAMPLE 1

A charge is made to a 1-1. stirred autoclave consisting of 1 mole (129 g) of dibutylamine, 1 mole of 2-chlorobenzaldehyde (140 g), 25 g of a 35 wt. % Cu-containing catalyst, prepared as described in U.S. Pat. No. 4,119,790, as a powder, and 350 ml of isopropanol.

The reactor is purged well with nitrogen, released to atmospheric pressure, and the reactants are heated to 95° C. The vapor pressure at this point is recorded. Acetylene then is admitted at a pressure of 100 psig above the recorded pressure. The amount of acetylene furnished to the reaction is measured by the loss in weight of the supply cylinder.

After about 12 hrs., corresponding to the absorption of 1 mole of acetylene (26 g), the reactor is cooled and the product is discharged. The reaction mixture is filtered to remove catalyst and stripped of solvent by rotary evaporation. Gas chromatographic analysis of the resulting crude reaction product mixture indicates it contains about 65% 3-dibutylamino-3-(2-chlorophenyl)-prop-1-yne. The crude mixture then is purified by molecular distillation at  $130\text{--}140^\circ\text{ C}$ . at about 0.1 mm to give the purified compound. Gas chromatographic assays indicates that the compound has a purity of at least 84%. The IR spectra shows a sharp band at  $3340\text{ cm}^{-1}$ ; and the NMR spectrum contains distinctive doublets at  $5.1$  and  $2.9\delta$  in addition to absorptions associated with the butyl and 2-chlorophenyl groupings.

#### EXAMPLES 2-6

Using the same procedure as described in Example 1 except that a charge of the dialkylamine and substituted benzaldehyde appropriate for the desired acetylenic amines is used, the following compounds listed below are obtained. Their purity by GC analysis, boiling point, and distinctive absorptions in the IR ( $\text{cm}^{-1}$ ) and NMR ( $\delta$ ) associated with  $>\text{CHC}\equiv\text{CH}$  are indicated.

- (2) Dimethylamino-3-(4-chlorophenyl)-prop-1-yne; 84%; ir  $3320\text{ cm}^{-1}$ ; nmr 4.55(d) and 2.6(d).
- (3) Dibutylamino-3-(4-methylphenyl)-prop-1-yne; 94.7%,  $160^\circ/1\text{ mm}$ . ir;  $3330\text{ cm}^{-1}$ ; nmr 4.8 and 2.3(d).
- (4) Dibutylamino-3-(4-methoxyphenyl)-prop-1-yne; 95.3%;  $137^\circ/0.5\text{ mm}$ ; ir  $3320\text{ cm}^{-1}$ ; nmr 4.78(d) and 2.45(d).
- (5) Dibutylamino-3-(2,4-dichlorophenyl)-prop-1-yne; and ir  $3320\text{ cm}^{-1}$ ; nmr 5.08(d) and 2.9(d).
- (6) Dibutylamino-3-(4-chlorophenyl)-prop-1-yne; 87%;  $131^\circ/0.8\text{ mm}$ ; ir  $3320\text{ cm}^{-1}$ ; nmr 4.8(d) and 2.4(c).

d=doublet

c=complex

The compounds of the present invention were tested in the usual way to determine their effectiveness as corrosion inhibitors. In such tests, strips of 1020 carbon steel of the dimensions  $2.5''\times 1.0''\times 0.20''$  were first degreased with methylethyl ketone and then descaled by soaking in 10% hydrochloric acid solution containing approximately 0.1% propargyl alcohol. The coupons then were cleaned with an acid brush and thoroughly rinsed with water. After rinsing, the coupons were soaked in 2% sodium carbonate solution, rinsed successively with water and acetone and air dried. The surface dimensions of the cleaned coupons were determined with the vernier scale and the coupons were allowed to dry in a desiccator. Before use the coupons were weighed on an analytical balance.

The tests were carried out in a 4 oz. jar containing a weighed amount of the inhibitor. The total solution

weight was taken to 100.0 g with the addition of 15% hydrochloric acid. The coupon then was then placed in the mixture and the jar loosely capped and placed in a 80° C. oil bath. After 16 hours the jar was removed from the oil bath and the contents were allowed to attain ambient conditions. The coupon was removed from the acid solution, thoroughly washed with water, 2% sodium carbonate solution, again with water, and finally rinsed with acetone. After air drying the coupon was kept in a desiccator before weighing and the net weight 10 loss was calculated by the established procedure.

A control also was run using no inhibitor whatsoever, and for comparative purposes, with dimethylamino-3-phenyl-prop-1-yne.

The test results are presented in the Table below, 15 where a lower value of weight loss represent good corrosion inhibition.

TABLE

## EFFECTIVENESS OF COMPOUNDS OF INVENTION AS CORROSION INHIBITORS

## Compound of Formula III

| R <sub>1</sub> & R <sub>2</sub> |  | Conditions of Test                 | Wt. Loss (%) |
|---------------------------------|-----------------------------------------------------------------------------------|------------------------------------|--------------|
| Butyl                           | 2-Chlorophenyl                                                                    | 0.4% Inhibitor; 15% HCl; 16 hrs.   | 0.03         |
| Butyl                           | 4-Chlorophenyl                                                                    | 0.4% Inhibitor; 15% HCl; 16 hrs.   | 0.03         |
| Butyl                           | 4-Methylphenyl                                                                    | 0.4% Inhibitor; 15% HCl; 16 hrs.   | 0.06         |
| Butyl                           | 4-Methoxyphenyl                                                                   | 0.4% Inhibitor; 15% HCl; 16 hrs.   | 0.11         |
| Butyl                           | 2,4-Dichlorophenyl                                                                | 0.4% Inhibitor; 15% HCl; 16 hrs.   | 0.04         |
| No Inhibitor                    |                                                                                   | 0.4% Inhibitor; 15% HCl; 16 hrs.   | 26.50        |
| Butyl                           | 4-Chlorophenyl                                                                    | 0.2% Inhibitor, 15% HCl; 16 hrs.   | 0.06         |
| Methyl                          | 4-Chlorophenyl                                                                    | 0.4% Inhibitor; 15% HCl; 16 hrs.   | 0.08         |
| Methyl                          | Phenyl*                                                                           | 0.4% Inhibitor; 15% HCl; 16 hrs.   | 0.87         |
| No Inhibitor                    |                                                                                   | 0.4% Inhibitor; 37.5% HCl; 4 hrs.  | 0.17         |
| Butyl                           | 2-Chlorophenyl                                                                    | 0.4% Inhibitor; 37.5% HCl; 4 hrs.  | 0.29         |
| Butyl                           | 4-Methylphenyl                                                                    | 0.4% Inhibitor; 37.5% HCl; 4 hrs.  | 0.55         |
| Butyl                           | 4-Methoxyphenyl                                                                   | 0.4% Inhibitor; 37.5% HCl; 4 hrs.  | 0.41         |
| Butyl                           | 2,4-Dichlorophenyl                                                                | 0.4% Inhibitor; 37.5% HCl; 4 hrs.  | 0.44         |
| No Inhibitor                    |                                                                                   | 0.4% Inhibitor; 37.5% HCl; 4 hrs.  | 0.48         |
| Butyl                           | 4-Chlorophenyl                                                                    | 0.4% Inhibitor; 37.5% HCl; 16 hrs. | 1.30         |
| Butyl                           | 4-Methylphenyl                                                                    | 0.4% Inhibitor; 37.5% HCl;         | 0.85         |

## TABLE-continued

## EFFECTIVENESS OF COMPOUNDS OF INVENTION AS CORROSION INHIBITORS

| Compound of Formula III | R <sub>1</sub> & R <sub>2</sub> |  | Conditions of Test                         | Wt. Loss (%) |
|-------------------------|---------------------------------|------------------------------------------------------------------------------------|--------------------------------------------|--------------|
| Butyl                   | 4-Methoxyphenyl                 |                                                                                    | 16 hrs. 0.4% Inhibitor; 37.5% HCl; 16 hrs. | 1.07         |
| Butyl                   | Phenyl*                         |                                                                                    |                                            | 4.23         |
| No Inhibitor            |                                 |                                                                                    |                                            | 54.90        |
| Methyl                  | 4-Chlorophenyl                  |                                                                                    | 0.4% Inhibitor; 37.5% HCl; 16 hrs.         | 10.83        |
| Methyl                  | Phenyl*                         |                                                                                    | 0.4% Inhibitor; 37.5% HCl; 16 hrs.         | 14.55        |
| No Inhibitor            |                                 |                                                                                    |                                            | 54.90        |

\*Comparative tests

As is seen from the data in the Table, the substituted-phenyl compounds of the invention exhibit excellent corrosion inhibition for metal in aqueous acid solution. These compounds perform substantially better than the corresponding unsubstituted phenyl compounds, even in different concentrations of acid and for various periods of exposure.

While the invention has been described with reference to certain embodiments thereof, it will be understood that modifications and changes may be made which are within the skill of the art. Accordingly, it is intended to be bound by the following claims in which:

We claim:

1. An aqueous composition for inhibiting the corrosion of metals placed therein comprising:

(a) an effective amount of a corrosion-inhibiting compound having the formula:



where

R<sub>1</sub> and R<sub>2</sub> are independently alkyl C<sub>1</sub>-C<sub>8</sub>; R<sub>3</sub> is independently halo, alkyl C<sub>1</sub>-C<sub>8</sub>, or alkoxy C<sub>1</sub>-C<sub>8</sub>; and n is 1 or 2; and

(b) a non-oxidizing acid.

2. A composition according to claim 1 wherein R<sub>3</sub> in said compound is halo.

3. A composition according to claim 1 wherein R<sub>3</sub> in said compound is chloro.

4. A composition according to claim 1 wherein R<sub>3</sub> in said compound is alkyl C<sub>1</sub>-C<sub>8</sub>.

5. A composition according to claim 1 wherein R<sub>3</sub> is alkoxy C<sub>1</sub>-C<sub>8</sub>.

6. A composition according to claim 1 wherein both R<sub>1</sub> and R<sub>2</sub> are the same.

7. A composition according to claim 1 wherein n is 1.

8. A composition according to claim 1 wherein n is 2.

9. A composition according to claim 1 in which said compound is a 3-dialkylamino-3-(2-chlorophenyl)-prop-1-yne.

10. A composition according to claim 1 in which said compound is a 3-dialkylamino-3-(2,4-dichlorophenyl)-prop-1-yne.

11. A composition according to claim 1 in which said compound is a 3-dialkylamino-3-(4-alkylphenyl)-prop-1-yne.

12. A composition according to claim 1 in which said compound is a 3-dialkylamino-3-(4-methoxyphenyl)-prop-1-yne.

13. A composition according to claim 1 in which said compound is 3-dibutylamino-3-(2-chlorophenyl)-prop-1-yne.

14. A compound of the formula:



where

$\text{R}_1$  and  $\text{R}_2$  are independently alkyl  $\text{C}_1\text{--C}_8$ ;

8  
 $\text{R}_3$  is independently halo, alkyl  $\text{C}_1\text{--C}_8$  or alkoxy  $\text{C}_1\text{--C}_8$ ; and  
 $n$  is 1 or 2.

15. A compound according to claim 14 wherein  $\text{R}_3$  is halo.

16. A compound according to claim 14 wherein  $\text{R}_3$  is chloro.

17. A compound according to claim 14 wherein  $\text{R}_3$  is alkyl  $\text{C}_1\text{--C}_8$ .

18. A compound according to claim 14 wherein  $\text{R}_3$  is alkoxy  $\text{C}_1\text{--C}_8$ .

19. A compound according to claim 14 wherein both  $\text{R}_1$  and  $\text{R}_2$  are the same.

20. A compound according to claim 14 wherein  $n$  is 1.

21. A compound according to claim 14 wherein  $n$  is 2.

22. A compound according to claim 14 which is a 3-dialkylamino-3-(2-chlorophenyl)-prop-1-yne.

23. A compound according to claim 14 which is a 3-dialkylamino-3-(2,4-dichlorophenyl)-prop-1-yne.

24. A compound according to claim 14 which is a 3-dialkylamino-3-(4-alkylphenyl)-prop-1-yne.

25. A compound according to claim 14 which is a 3-dialkylamino-3-(4-methoxyphenyl)-prop-1-yne.

26. A compound according to claim 14 which is 3-dibutylamino-3-(2-chlorophenyl)-prop-1-yne.

\* \* \* \* \*

30

35

40

45

50

55

60

65